

# UNITED STATES PATENT OFFICE.

LEON CAMMEN, OF NEW YORK, N. Y.

## CENTRIFUGAL CASTING.

1,410,885.

Specification of Letters Patent. Patented Mar. 28, 1922.

No Drawing.

Application filed August 12, 1921. Serial No. 491,845.

To all whom it may concern:

Be it known that I, LEON CAMMEN, a citizen of the United States, and resident of borough of Manhattan, in the city, county, and State of New York, have invented certain useful and new Improvements in Centrifugal Castings, of which the following is a specification.

The present invention refers to the production of centrifugal castings from metals which chill rapidly from the molten state, as e. g. monel metal or high-chromium steel.

In the past (with the exception of the practice of the present inventor) the molds in centrifugal casting were used either at room temperature or warmed up only slightly, enough to take off the chill of the mold and to ensure its being dry. In fact the present inventor knows of no case where the mold was heated higher than 300 to 400 deg. F. As a result of this, it has not proved hitherto possible to produce good and sound centrifugal castings of such metals as monel in tubes of small diameters, such as 3 to 4 in., which I have done successfully by my method.

A brief thermodynamic calculation will show the reasons for the failure to do so. Assume that it is desired to cast a tube 60 in. long, 3 in. outside and 2.5 in. inside diameter. Such a tube in monel metal weighs roughly 60 lb. If before casting the metal is heated to a temperature say 200 deg. above the melting point (and is not safe to go beyond that), the metal will contain roughly (specific heat of monel metal 0.12) 1500 B. t. u. of heat that it can lose before it reaches the temperature of initial congealation.

But the mold, made up of a refractory material and some metal like steel, must be at least 1.5 in. thick, which means that it will have a volume of at least 600 cu. in. and a combined weight of about 120 to 150 lb. Assuming the lower figure, and a combined specific heat of 0.10, which is certainly low, one can easily see that if while the metal is being poured, the average temperature of the mold is raised more than 125 deg., enough heat is abstracted to congeal the metal.

From this it clearly appears that, unless the metal is poured so rapidly that it will assume a form of a tube due to centrifugal spinning before the mold is heated up to 125 deg. F. above its initial temperature, it

is impossible to cast a good tube of the dimensions indicated above. As hitherto no way has been discovered to pour the metal with the rapidity required, and as with the usual methods of pouring and a mold at room temperature, the temperature of the mold during pouring rises several hundred degrees, it has proved to be impossible to make small tubing of such metals as monel in cold molds.

The same calculation explains why heating the mold to say 300 or 400 deg. F., as is frequently done now, is of no avail in this connection. As monel metal is being poured into the mold at say 2700 deg. F., the difference between an initial temperature of the mold of say 100 and 400 deg. is scarcely material, the rise of temperature of the mold being of the order of 700 to 1000 deg. F., i. e. considerably beyond the limits which are safe if it is desired to maintain the metal after pouring in a fluid condition long enough to permit it to form a good tube.

In this connection it should be mentioned that it is by no means sufficient to maintain the metal fluid long enough for it to acquire a tubular shape before it solidifies. In centrifugal casting the venting of the mold is naturally very poor, and the only way the gases in the metal have for their escape is towards the center of the mold, or tube, this being materially assisted by the tendency of the metal to pack tight under the action of centrifugal force. But the only way the gases can thus escape is providing the metal remains fluid long enough to permit them to do so. If therefore the metal congeals too rapidly, there may be a tubular shape cast, but the metal will be full of blowholes and porosity.

To avoid this, the present inventor resorts to a heating of the mold to a very high temperature, in excess of 1000 deg. F., and preferably to about 2000 deg. F. for monel metal and steel, and in general, preferably to a temperature not less than one half the melting temperature of the metal to be cast, as expressed in degrees of the Fahrenheit thermometric scale, so that e. g. for bronze, melting at 1700 deg. F., the heating of the mold to say 850 deg. would be sufficient, though the employment of a somewhat higher temperature, say 1000 deg. F. is recommended.

This heating may be done in various ways,

as by placing the mold into a furnace, passing an electric current through the mold, etc.

I claim:

5. 1. A process of centrifugal casting wherein, previous to the pouring of the metal, the mold is by external means other than the metal of the casting heated to a temperature, in degrees Fahrenheit scale, not less than 10 one-half that of the melting point of the metal of the goods cast.
2. A process of centrifugal casting of monel metal or steel wherein the mold, previous to the pouring of the metal, is by external means other than the metal of the casting heated to a temperature not less than 1000 deg. F.
3. A process of centrifugal casting of bronze wherein the mold previous to the pouring of the metal, is by external means other than the metal of the casting heated to a temperature not less than 850 deg. F.
4. A process of centrifugal casting wherein, previous to the pouring of the metal, the

mold is by external means other than the 25 metal of the casting heated to such a temperature that the loss of heat from the metal to the mold at its obtaining temperature be less than that which is sufficient to chill the metal to the point of congelation within the time period necessary for the formation of the proper casting shape and for the escape of the gases from the metal.

5. A process of centrifugal casting wherein, previous to the pouring of the metal, the 35 mold is by external means other than the metal of the casting heated to such a temperature that the loss of heat from the metal to the mold at its obtaining temperature be less than that which is sufficient to chill the metal to the point of congelation within the time period necessary for the formation of the proper casting shape.

Signed in New York, in the county and State of New York, August 10th, A. D. 1921. 45  
LEON CAMMEN.

Witness:

LOUISE REINSCHMIDT.